

# United States Patent

Aggen

[15] 3,650,731

[45] Mar. 21, 1972

## [54] FERRITIC STAINLESS STEEL

[72] Inventor: George Aggen, Sarver, Pa.

[73] Assignee: Allegheny Ludlum Steel Corporation, Pittsburgh, Pa.

[22] Filed: Jan. 31, 1969

[21] Appl. No.: 795,740

[52] U.S. Cl. 75/128 T, 75/125, 75/128 T,  
75/128 V

[51] Int. Cl. C22c 39/20

[58] Field of Search 75/126 R, 125

## [56] References Cited

### UNITED STATES PATENTS

|           |         |        |          |
|-----------|---------|--------|----------|
| 2,056,765 | 10/1936 | Becket | 75/126 R |
| 2,590,835 | 4/1952  | Kirkby | 75/126 R |
| 2,848,323 | 8/1958  | Harris | 75/126 R |

|           |        |         |          |
|-----------|--------|---------|----------|
| 3,000,729 | 9/1961 | Tanczyn | 75/126 R |
| 3,250,611 | 5/1966 | Lulg    | 75/126 R |
| 3,490,956 | 1/1970 | Wilton  | 75/126 R |

Primary Examiner—Hyland Bizot

Attorney—Richard A. Speer and Vincent G. Gioia

[57]

## ABSTRACT

A hot rolled ferritic stainless steel having up to 0.07% carbon, 10–12.5% chromium, traces to 0.75% silicon, traces to 3% manganese, traces to 2% copper, 0.5 to 1.5% nickel, 0.1 to 0.5% titanium and which may contain as small alloying additions aluminum, vanadium, zirconium, columbium or combinations thereof. The elements of the steel are also balanced with respect to each other so that it is capable of being softened to  $R_b$  80 hardness or lower in less than about 24 hours of subcritical box annealing and develops at least 50% austenite during hot rolling so as to exhibit a charpy V-notch impact strength of at least 20 ft.-lb. at 0° F.

2 Claims, No Drawings

## FERRITIC STAINLESS STEEL

A few years ago a ferritic stainless steel was developed which possesses the attractive features of low cost, good formability, good weldability and adequate corrosion resistance for many applications. However, this alloy, which is known commercially as MF-1, (described in U.S. Pat. No. 3,250,611) has a relatively low strength (about 40 k.s.i. yield strength) unless cold worked and a high impact transition temperature, i.e., about 70° F. At 0° F. this alloy generally has a charpy V-notch impact strength of about 4 ft.-lb. The high impact transition temperature in particular detracts from its usefulness for certain structural applications. It is desirable, therefore, to improve the strength and toughness of MF-1 type steels without adversely affecting the steel's other beneficial properties and without unduly increasing its cost.

The present invention provides an improved ferritic stainless steel having superior toughness and improved strength while maintaining adequate formability. Formability is conveniently measured by the hardness of the alloy and ferritic stainless steels in accordance with the invention are capable of being softened to a  $R_B$  hardness of 80 (or lower) in less than about 24 hours by subcritical box annealing, thus avoiding the necessity for unduly costly heat treatments. The strength level of the improved ferritic stainless steel in accordance with the invention is not obtained by cold working and thus is not limited to certain product forms such as those which would not have the effects of cold working destroyed by certain fabrication procedures, e.g., welding. In accordance with the invention there is provided a ferritic stainless steel consisting essentially of up to 0.1% carbon, preferably less than 0.07% carbon, up to 0.75% silicon, preferably 0.2 to 0.6%, up to 3% manganese, traces to 1.5% nickel, up to 2% copper, up to 0.8% of any of titanium, aluminum, vanadium, zirconium, and up to 1% columbium; said elements being balanced to provide a chromium equivalency ( $Cr_E$ ) of not greater than 10 according to the following equation:

$$Cr_E = \%Cr + 1.5(\%Si) + (\%Ti) + 2.5(\%A1) + 3(\%Cb) + 10(\%Zr) + 2(\%V) - 40(\%C+N) - 3(\%Ni) - 2(\%Mn+Cu);$$

so as to develop at least about 50% austenite (by volume) at hot rolling temperatures in the range of 1,600°-2,200° F. and attain an impact strength of at least 20 ft.-lb. at 0° F.; said steel being capable of softening to  $R_B$  80 or lower by subcritical box annealing in less than about 24 hours.

As described above, it is necessary that the elements in the steel in accordance with the invention be controlled and balanced in order to achieve the desired combination of properties characteristic of the invention. Thus, for example, the chromium must be present in a quantity of at least 10% to assure satisfactory corrosion resistance and addition of this element beyond about 12.5% is an unnecessary expense, as the additional corrosion resistance provided is not required for many applications. The chromium level in the present invention is similar to that of MF-1 type steels. In the same manner

the limits on carbon and silicon are comparable to that for the MF-1 type steels and for the same reasons. In the MF-1 steels titanium is added to combine with carbon to result in a low matrix carbon content so as to improve ductility and to help assure the ferritic character of the steel. In the present invention it is desired to improve toughness and accordingly the elements must be balanced to achieve this result. This can be accomplished by additions of up to about 3% manganese, up to about 2% copper or with small but effective amounts of nickel in an amount of from 0.5 to 1.5%. It can also be accomplished by substituting aluminum, vanadium or columbium or combinations of these elements for titanium. Substitutions are preferably at least about 0.05%. Additions of manganese or copper or nickel or combinations thereof decidedly lower the chromium equivalency of resulting alloys. When an alloy contains sufficient amounts of these elements the chromium equivalency will be below 10 insuring the formation of at least about 50% austenite at hot rolling temperatures within the range of 1,600°-2,200° F. and the attainment of good toughness. Nickel content, however, must not exceed about 1.5% or the alloy will not possess adequate formability. It will not be capable of being softened to an  $R_B$  hardness of 80 or lower in less than about 24 hours of subcritical box annealing. Carbon and nitrogen can serve in the same manner as manganese, copper and nickel but are undesirable since they result in the formation of a hard and brittle martensite which can pose processing difficulties and welding problems. Aluminum, vanadium and columbium are weaker ferrite formers than titanium or zirconium which behaves similarly to titanium and therefore do not hinder the formation of austenite at hot rolling temperatures to the same degree as does titanium or zirconium. They are, however, effective carbide or nitride formers as are titanium and zirconium and may be useful in minimizing the formation of hard brittle martensite. Hence, through balancing of elements the present invention provides many of the advantages of the MF-1 type steels including relatively low cost and excellent formability plus the additional advantage of materially improved toughness, i.e., an improvement in the impact transition temperature from about 70° F. for MF-1 to below about 0° F.

Corrosion tests have proven that the steels in accordance with the present invention have corrosion resistance roughly comparable to the MF-1 type steels. The zirconium containing compositions appear to have a somewhat improved resistance to corrosion in atmospheric and salt spray tests.

The following examples will illustrate the practice of the invention in accordance with presently preferred embodiments. Also described below are comparative results with steels outside the limits set forth above.

Fifty pound heats were melted in an argon atmosphere. The argon was used to simulate the cleanliness and gas contents obtained during normal arc-furnace melting of commercial heats. An analysis of the heats is found below in Table I.

TABLE I

| Heat No. | C    | Mn   | P    | S    | Si  | Cr    | Ni   | N                  | Ti  | Al   | V | Cb | Cu | Zr  |
|----------|------|------|------|------|-----|-------|------|--------------------|-----|------|---|----|----|-----|
| RV-1787  | .043 | .50  | .015 | .011 | .39 | 11.25 | .24  | .010               | .52 |      |   |    |    |     |
| RV-1788  | .046 | .54  | .013 | .012 | .42 | 11.15 | .21  | .023               | .24 |      |   |    |    |     |
| RV-1770  | .044 | .49  | .008 | .010 | .50 | 11.40 | .23  | .006               |     |      |   |    |    | .47 |
| RV-1780  | .045 | .54  | .013 | .011 | .39 | 11.20 | .22  | .021               |     |      |   |    |    |     |
| RV-1781  | .050 | .50  | .013 | .011 | .36 | 11.15 | .22  | .023               |     |      |   |    |    | .46 |
| RV-1768  | .048 | .48  | .009 | .009 | .5  | 11.62 | .23  | .022               | .50 |      |   |    |    |     |
| RV-1771  | .050 | .48  | .010 | .010 | .5  | 11.18 | .23  | .008               |     |      |   |    |    | .99 |
| RV-1782  | .045 | .55  | .012 | .009 | .42 | 11.18 | .21  | .006               |     |      |   |    |    | .36 |
| RV-1783  | .046 | .54  | .013 | .010 | .42 | 11.22 | .21  | .007               |     |      |   |    |    | .92 |
| RV-1786  | .045 | .49  | .013 | .009 | .41 | 11.35 | .25  | .013               | .38 | .25  |   |    |    |     |
| RV-1784  | .048 | .53  | .015 | .010 | .42 | 11.10 | .22  | .008               | .27 |      |   |    |    | .48 |
| KA11     | .031 | .36  | .008 | .014 | .22 | 11.69 | .62  | .024               | .23 |      |   |    |    |     |
| KA26     | .022 | .36  | .008 | .018 | .18 | 11.60 | .97  | .019               | .32 |      |   |    |    |     |
| KA29     | .024 | .35  | .009 | .018 | .17 | 11.64 | 1.49 | <sup>1</sup> .0175 | .27 |      |   |    |    |     |
| KA30     | .022 | .37  | .009 | .011 | .18 | 11.62 | 2.02 | <sup>1</sup> .0175 | .29 |      |   |    |    |     |
| KG89     | .024 | .29  | .010 | .012 | .17 | 11.48 | 1.5  | <sup>1</sup> .0175 | .38 | .043 |   |    |    |     |
| KG93     | .029 | .28  | .012 | .013 | .18 | 11.60 | .98  | <sup>1</sup> .0175 | .37 | .041 |   |    |    | .97 |
| KG61     | .024 | 1.03 | .010 | .016 | .12 | 11.44 | 1.49 | <sup>1</sup> .0175 | .40 | .078 |   |    |    |     |
| KG57     | .023 | 2.02 | .011 | .014 | .16 | 11.68 | .01  | <sup>1</sup> .0175 | .39 | .024 |   |    |    |     |
| KG68     | .023 | .34  | .010 | .015 | .10 | 11.46 | .98  | <sup>1</sup> .022  |     | .075 |   |    |    |     |
| KG75     | .023 | .34  | .010 | .018 | .10 | 11.36 | 1.44 | <sup>1</sup> .022  |     | .096 |   |    |    |     |
| KG45     | .023 | .34  | .010 | .018 | .10 | 11.22 | 1.46 | <sup>1</sup> .022  |     | .170 |   |    |    |     |

<sup>1</sup> Estimated average depending on whether Ti or Al or Ti and Al present.

TABLE III  
[Charpy V-Notch Impact, ft.-lbs., at indicated temperatures]

| Heat No. | Degrees F. |         |         |         |         |        |         |       |         |
|----------|------------|---------|---------|---------|---------|--------|---------|-------|---------|
|          | -100       | -50     | -25     | 0       | 32      | 78-80  | 125     | 170   | 212     |
| RV-1787  |            |         |         | 4/4     | 3/5     | 6/6    | 9/11    | 23/30 | 195/212 |
| RV-1788  | 38/84      | 114/114 | 160/217 | 132/145 | 217/233 |        |         |       | 208/225 |
| RV-1770  | 4/5        | 6/8     | 36/136  | 218/219 | 211/220 |        |         |       | 196/218 |
| RV-1780  | 107/213    | 210/215 | 196/223 | 195/200 | 225/227 |        |         |       | 218/227 |
| RV-1781  | 90/186     | 175/216 | 195/214 | 222/226 | 210     |        |         |       | 196/210 |
| RV-1768  | 2/2        | 2/50    | 29/83   | 200/224 | 158/221 |        |         |       | 190/003 |
| RV-1771  |            |         | 4/4     | 4/5     | 4/6     | 6/8    | 12/12   |       | 17/19   |
| RV-1782  |            |         | 2       | 3/4     | 7/9     | 19/34  | 212/214 |       | 192/227 |
| RV-1783  |            |         | 2/3     | 3/3     | 5/6     | 18     | 19/27   |       | 37/41   |
| RV-1786  |            |         | 2/4     | 3/4     | 5/11    | 16/17  | 30/45   |       | 205/210 |
| RV-1784  |            |         | 4/4     | 5/5     | 1/10    | 18/215 | 50/183  |       | 183/212 |
| KA11     | 10.5       | 47.5    |         | 54.5    |         | 57.0   |         |       | 63.0    |
| KA26     | 20.5       | 59.0    |         | 65.5    |         | 108.5  |         |       | 114.5   |
| KA29     | 7.0        | 43.0    |         | 42.5    |         | 44.0   |         |       | 53.0    |
| KA30     | 4.0        | 12.0    |         | 41.0    |         | 48.5   |         |       | 72.0    |
| KA11     | 36.0       | 48.0    |         | 59.0    |         | 60.5   |         |       | 77.0    |
| KA26     | 18.0       | 37.0    |         | 82.0    |         | 88.0   |         |       | 109.5   |
| KA**29   | 12.0       | 41.0    |         | 62.0    |         | 101.0  |         |       | 122.5   |
| KA**30   | 67.5       | 101.0   |         | 114.0   |         | 119.0  |         |       | 130.0   |
| KG**89   | 16.0       | 118.0   |         | 136.0   |         | 190.5  |         |       |         |
| KG**93   | 11.0       | 16.0    |         | 40.0    |         | 134.5  |         |       |         |
| KG**61   | 41.0       | 113.0   |         | 178.0   |         | 197.0  |         |       |         |
| KG**57   | 140.0      | 125.0   |         | 181.0   |         | 199.5  |         |       |         |
| KG**68   | 4/4        | 22/107  |         | 215/230 |         |        |         |       |         |
| KG75***  | 25/61      | 64/88   |         | 58/108  |         |        |         |       |         |
| KG**45   | 6/7        | 210/230 |         | 228/230 |         |        |         |       |         |

<sup>1</sup> Average of two values 67 and 13.

All the heats except for RV-1787, RV-1771, RV-1782, RV-1783, RV-1786, RV-1784 and KA30 are within the scope of the present invention. Heat KA30 is outside the invention because of high nickel, over about 1.5%, and the others are outside the invention because of chromium equivalencies in excess of 10. The chromium equivalency for all the heats is given below in Table II. Attention is directed to heat RV-1787 which is a typical MF-I heat.

TABLE II

| Heat No. | Chromium Equivalency |
|----------|----------------------|
| RV-1787  | 11.74                |
| RV-1788  | 7.91                 |
| RV-1770  | 9.89                 |
| RV-1780  | 7.88                 |
| RV-1781  | 8.03                 |
| RV-1768  | 9.07                 |
| RV-1771  | 10.93                |
| RV-1782  | 11.64                |
| RV-1783  | 17.26                |
| RV-1786  | 11.12                |
| RV-1784  | 13.24                |
| KA11     | 9.20                 |
| KA26     | 8.80                 |
| KA29     | 6.91                 |
| KA30     | 5.60                 |
| KG89     | 5.91                 |
| KG93     | 6.25                 |
| KG51     | 6.51                 |
| KG57     | 5.99                 |
| KG68     | 6.37                 |
| KG75     | 4.94                 |
| KG45     | 4.94                 |

All the heats found in Table I were hot worked and annealed. More particularly the RV series were pressed to 1½-inch squares from 2,200° F., hot rolled to ¼-inch bars from 1,950° F. and annealed for one-half hour at 1,500° F. The KA series were pressed to slabs 2 × 5 inches from 2,350° F., hot rolled from 2,225° F. to ½-inch thickness, reheated to 1,525° F. and hot rolled at 1,525° F. in one pass to a ¼-inch thickness. KA samples belonging to the KA\* series, see Table III, were additionally annealed at 1,200° F. for 1 hour and KA samples belonging to the KA\*\* series were additionally annealed at 1,400° F. for 1 hour. The KG series samples were forged to 1½-inch from 2,000° F., reheated and forged to ¼-inch bars with a finishing temperature below 1,500° F. and annealed. The KG samples belonging to the KG\* series were annealed for one-half hour at 1,500° F. and air cooled while KG samples belonging to the KG\*\* series were annealed for 1 hour at 1,350° F. and air cooled. The KG sample belonging to the KG\*\*\* series was annealed by holding for 1 hour at 1,550° F., furnace cooling to 1,200° F. and air cooling to room temperature.

Table III below summarizes the results of charpy V-notch impact tests carried out over a range of temperatures for the samples whose compositions are given in Table I.

It is noted that all the alloys attained a charpy V-notch impact strength of at least 20 ft-lb. at 0° F. except for those singled out earlier for having chromium equivalencies in excess of 10. These are the alloys which do not develop at least about 50% austenite (by volume) at hot rolling temperatures in the range of 1,600°-2,200° F. For example, heat RV-1783 containing in excess of 0.8% zirconium is fully ferritic and hence exhibits a high impact transition temperature.

As stated earlier the alloys in accordance with the invention are capable of being softened to an  $R_B$  hardness of 80 in less than about 24 hours by subcritical box annealing. The ability to be softened is an important factor for good formability. To insure satisfactory formability the nickel content must be maintained below about 1.5%. In order to show the criticality of nickel, 50 pound heats of KA11, KA26, KA29 and KA30, whose compositions can be found in Table I, were processed by pressing to 2×5-inch slabs from 2,350° F., hot rolling to 0.150 inch from 2,225° F., annealing for 15 minutes at 1,500° F., cold rolling to 0.090 inch and final annealing for 5 minutes. Final annealing temperatures are shown in Table IV along with the members hardness values. It is noted that member KA30 which contains more than 1.5% nickel, could not be softened sufficiently so as to attain good formability, even with treatments known to provide maximum softness. Members KA11, KA26 and KA29 showed that alloys containing from about 0.5% to about 1.5% nickel, up to 0.07% carbon and from 0.1 to 0.5% titanium could attain a charpy V-notch impact strength of at least 20 ft-lb. at 0° F. and could be softened. Of course, alloys with nickel levels in excess of residual amounts and less than 0.5%, i.e., about 0.35%, can also be softened.

60

TABLE IV

| Heat No.           | Anneal Temp. °F. | Hardness $R_B$ |
|--------------------|------------------|----------------|
| KA11<br>(0.52% Ni) | 1300             | 75             |
|                    | 1400             | 73             |
|                    | 1500             | 73             |
| KA26<br>(0.97% Ni) | 1400             | 73             |
|                    | 1500             | 73             |
|                    | 1600             | 80             |
| KA29<br>(1.49% Ni) | 1300             | 77             |
|                    | 1400             | 76             |
| KA30<br>(2.02% Ni) | 1300             | 92.5           |
|                    | 1500             | 94             |
|                    | 1600             | 99             |

Four additional heat treatments were performed with KA30 to see if it could be softened below  $R_B$ 80. Found below in Table V are the heat treatments along with the respective hardness values obtained.

TABLE V

|                                                                                                                          |      |
|--------------------------------------------------------------------------------------------------------------------------|------|
| A. (a) anneal at 2000° F. for 10 min.<br>(b) water quench                                                                | 26.3 |
| B. (a) anneal at 2000° F. for 10 min.<br>(b) furnace cool at 100° F. per<br>hour to below 1000° F.<br>(c) air cool       | 25.8 |
| C. (a) anneal at 2000° F. for 10 min.<br>(b) transfer to furnace at 1400° F.<br>and hold 16-24 hours<br>(c) water quench | 27.3 |
| D. (a) anneal at 2000° F. for 10 min.<br>(b) transfer to furnace at 1200° F.<br>and hold 16-24 hours<br>(c) water quench | 26.8 |

It is noted for contrast that KA26 (1% Ni) given heat treatment B and D exhibits hardness of  $R_B$ 67.7 and  $R_B$ 71.5.

It will be apparent to those skilled in the art that the novel principles of the invention disclosed herein in connection with specific examples thereof will suggest various other modifica-

tions and applications of the same. It is accordingly desired that in construing the breadth of the appended claims they shall not be limited to the specific examples of the invention described herein.

5 I claim:

1. A hot rolled ferritic stainless steel consisting essentially of, in weight percent, up to 0.07% carbon, 10-12.5% chromium, up to 0.75% silicon, up to 3% manganese, 0.5 to 1.5% nickel, 0.1 to 0.5% titanium, up to 0.8% aluminum, up to 1.0% columbium, up to 0.8% zirconium, up to 0.8% vanadium, up to 2% copper, balance essentially iron, said elements being balanced to provide a chromium equivalency ( $Cr_E$ ) of not greater than 10 according to the following equation:

$$15 \quad Cr_E = \frac{Cr + 1.5(Si) + (Ti) + 2.5(A1)}{+3(Cb) + 10(Zr) + 2(V) - 40(C + N) - 3(Ni) - 2(Mn + Cu)}$$

so as to be capable of developing at least 50% austenite (by volume) at hot rolling temperatures in the range of 1,600°-2,200° F. and attaining a charpy V-notch impact strength of at least 20 ft.-lb. at 0° F., said steel being capable of softening to  $R_B$ 80 by subcritical box annealing in less than about 24 hours.

20 2. A ferritic stainless steel according to claim 1 having 0.2 to 0.6% silicon.

25 \* \* \* \* \*

30

35

40

45

50

55

60

65

70

75